

## UNITED STATES PATENT OFFICE

2,027,995

STRONG PERMANENT MAGNET WITH TUNG-  
STEN, MOLYBDENUM, OR CHROMIUMTokushichi Mishima, Ochiai-machi,  
Toyotama-gori, Tokyo, JapanNo Drawing. Original application January 20,  
1932, Serial No. 587,822. Divided and this ap-  
plication May 31, 1933, Serial No. 673,795. In  
Japan March 9, 1931

8 Claims. (Cl. 175—21)

The invention relates to a strong permanent magnet and forms a divisional application to Serial No. 587,822 filed January 20, 1932.

In my co-pending application No. 587,822, I 5 fully explained a new permanent magnet comprising 5 to 40% Ni, 7 to 20% Al and the remainder substantially iron, with or without the addition of other metals, and carbon below 1.5% and also small impurities. The subject matter 10 of the invention is a division from the above mentioned application.

According to the invention it has been found 15 that by adding tungsten to the new alloy as mentioned above, the alloy can further be improved in its characteristic properties, giving a higher coercive force and a stronger residual magnetism, as well as a better malleability and ductility. In consequence the alloy is also suitable for making magnets required to be finished by complicated 20 and precise working. The amount of tungsten to be added is 0.5 to 8%. The tungsten makes the grain-size minute and serves to increase the number of the molecular magnets arranged irregularly at the boundary of the grains. It is 25 due to this fact that a high coercive force and good residual magnetism as well as good toughness can be obtained.

Actual examples for carrying out the invention thus modified are given below:

| Chemical composition (per cent) |        |                |          | Magnetic properties               |                                       |
|---------------------------------|--------|----------------|----------|-----------------------------------|---------------------------------------|
| Iron                            | Nickel | Alumin-<br>ium | Tungsten | Coercive<br>force (Hc)<br>(gauss) | Residual<br>magnetism<br>(Br) (gauss) |
| 70.3                            | 17.0   | 9.5            | 2.0      | 155                               | 9,700                                 |
| 68.5                            | 16.5   | 9.8            | 5.0      | 140                               | 9,200                                 |
| 62.0                            | 25.0   | 10.0           | 2.7      | 270                               | 9,650                                 |
| 55.5                            | 30.0   | 11.5           | 2.8      | 460                               | 9,500                                 |

It is also noted in this case that the presence of carbon of below 1.5% and/or a small amount of impurities does not materially affect the magnetic properties of the alloy.

According to the invention it has further been found that by adding molybdenum of below 10% to the new alloy as above, the alloy is further improved, because the molybdenum also makes the crystal grains minute and consequently increases the coercive force and the residual mag-

netism. Besides the forging property of the alloy is much improved.

Actual examples for this case are given below:

| Chemical composition (per cent) |        |                |                 | Magnetic properties               |                                       | 5  |
|---------------------------------|--------|----------------|-----------------|-----------------------------------|---------------------------------------|----|
| Iron                            | Nickel | Alumin-<br>ium | Molyb-<br>denum | Coercive<br>force (Hc)<br>(gauss) | Residual<br>magnetism<br>(Br) (gauss) | 10 |
| 65.0                            | 24.5   | 10.0           | 0.5             | 290                               | 9,600                                 |    |
| 62.0                            | 23.0   | 10.0           | 5.0             | 300                               | 9,400                                 |    |
| 56.0                            | 30.0   | 12.0           | 2.0             | 490                               | 9,500                                 |    |

In this case also it is noted that the presence 15 of carbon of below 1.5% and/or a small amount of impurities does not materially affect the magnetic properties of the alloy.

According to the invention it has further been 20 found that by adding 1 to 5% chromium and/or carbon of below 1.0%, to the new alloy as above mentioned, an alloy having a higher coercive force and a stronger residual magnetism can also be obtained.

Actual examples for this case are illustrated 25 below:

| Chemical composition (per cent) |        |                |        |        | Magnetic properties               |                                       | 30 |
|---------------------------------|--------|----------------|--------|--------|-----------------------------------|---------------------------------------|----|
| Iron                            | Nickel | Alumin-<br>ium | Chrome | Carbon | Coercive<br>force (Hc)<br>(gauss) | Residual<br>magnetism<br>(Br) (gauss) | 35 |
| Rest                            | 18.0   | 10.0           | 3.0    | 0.1    | 172                               | 10,000                                |    |
| 62.5                            | 24.8   | 10.0           | 2.3    | 0.2    | 265                               | 9,700                                 |    |
| 54.3                            | 30.5   | 12.0           | 3.0    | 0.2    | 500                               | 9,600                                 | 35 |

What I claim is:—

1. A permanent magnet comprising main and auxiliary elements, the main elements consisting 40 of nickel 5 to 40%, aluminum 7 to 20% and the remainder iron; the auxiliary elements consisting of one of the metals chromium from 1.0 to 5%, tungsten from 0.5 to 8% and molybdenum from trace to 10%.

2. A permanent magnet comprising main and auxiliary elements, the main elements consisting of nickel 5 to 40%, aluminum 7 to 20% and the remainder substantially iron; the auxiliary elements consisting of one of the metals chromium 45

50

from 1.0 to 5%, tungsten from 0.5 to 8% and molybdenum from trace to 10%.

3. A permanent magnet comprising nickel 5 to 40%, aluminum 7 to 20%, tungsten 0.5 to 8% and the remainder iron.

4. A permanent magnet comprising nickel 5 to 40%, aluminum 7 to 20%, tungsten 0.5 to 8%, carbon from trace to 1.5% and the remainder iron.

10 5. A permanent magnet comprising nickel 5 to 40%, aluminum 7 to 20%, molybdenum from trace to 10% and the remainder iron.

6. A permanent magnet comprising nickel 5 to 40%, aluminum 7 to 20%, molybdenum from trace to 10%, carbon from trace to 1.5% and the remainder iron.

7. A permanent magnet comprising nickel 5 to 40%, aluminum 7 to 20%, chromium 1 to 5% and the remainder iron.

8. A permanent magnet comprising nickel 5 to 40%, aluminum 7 to 20%, chromium 1 to 5%, carbon from trace to 1.0% and the remainder 10 iron.

TOKUSHICHI MISHIMA.